# EUROPEAN PATENT APPLICATION

(11) **EP 0 082 586 A2**
(43) Date of publication of application: **29.06.1983**
(21) Application number: 82304209.8
(22) Date of filing: 10.08.1982
(51) Int. Cl.: C10G 1/04

(54) **An improved process for the liquefaction of solid carbonaceous materials**

(30) Priority: 21.12.1981 US 332583
(71) Applicant: EXXON RESEARCH AND ENGINEERING COMPANY, Florham Park, New Jersey 07932-0390 (US)
(72) Inventor: Bauman, Richard Frank, Houston Texas (US)
(74) Representative: Pitkin, Robert Wilfred

(57) **Abstract**

An improved process for liquefying solid carbonaceous materials wherein liquefaction yields are increased by extracting the normally solid bottoms product with a solvent containing donatable hydrogen. The extraction is accomplished at a temperature within the range from about 50 to about 600°F and at a pressure within the range from about 0 to about 750 psig and at least a portion of the extract is recycled to the liquefaction reaction zone.

## Description

This invention relates to a process for converting coal or similar solid carbonaceous materials. More particularly, this invention relates to an improved process for liquefying coal and similar solid carbonaceous materials.

As is also well known, proven petroleum and gas reserves are shrinking throughout the world and the need for alternative sources of energy is becoming more and more apparent. One such alternative sourceis,of course, coal since coal is an abundant fossil fuel in many countries throughout the world. Before coal will be generally accepted by the ultimate consumer, however, it will be necessary to convert the same to a form which will permit use in those areas where liquid or gaseous fuels are normally required.

To this end, several processes wherein coal is either liquefied and/or gasified have been proposed heretofore. Of these, the processes wherein coal is liquefied appear to be more desirable since a broader range of products is produced and these products are more readily transported and stored.

Of these several liquefaction processes which have heretofore been proposed, those processes wherein coal is liquefied in the presence of a solvent or diluent, particularly a hydrogen-donor solvent or diluent, and in the presence of a hydrogen-containing gas appear to offer the greater advantages. In these processes, liquefaction is accomplished at elevated temperatures and pressures and hydrocarbon gases are invariably produced as by-products. For the most part, however, these and other liquefaction processes yield a normally solid bottoms product containing relatively large quantities of carbon, which bottom product cannot be discarded without further processing when an economic, waste-free process is sought. Heretofore, several methods have been proposed in an effort to avoid this deficiency. For example, the normally solid, bottoms product can be subjected to further liquefaction in a separate stage or stages until such time as the carbon content of the normally solid, bottoms product has been reduced to a point where the carbon content thereof is sufficiently low such that discarding thereof does not significantly and adversely affect the economics of the process. Staged liquefaction, however, significantly increases both investment and operating costs as a result of the additional equipment required and as a result of the energy and other utilities required to effect the further liquefaction. It has also been proposed, heretofore, to recycle all or a portion of the normally solid, bottoms product to a single or plural liquefaction stage. When this is done, however, a large portion of the material recycle is either unreactive (ash) or it is difficult to convert (fusinite). These materials can amount to 60% of the recycle material and recycle of these materials raises costs and lowers thermal efficiency. It has also been proposed, heretofore, to simply burn the normally solid, bottoms product, directly, or to gasify the normally solid, bottoms product to produce a gaseous product which can then be burned as a fuel. Operation in this manner, however, reduces the yield of normally liquid products, thereby reducing thermal efficiency, and increases both investment and operating costs for essentially the same reasons already noted with respect to staged or further liquefaction. Finally, it has been proposed, heretofore, to separate the unreactive and fusinite portions of the bottoms from-the reactive portion thereof by extraction. Generally, however, these operations depend upon the use of a relatively expensive solvent (such as toluene) which must then be separated from the extract, generally, by vaporization. This type of operation too has proven expensive due primarily to the high energy requirement for separation of the solvent.

In light of the foregoing, the need for a liquefaction process which can be operated in a mode requiring fewer liquefaction stages at an increased thermal efficiency to yield a normally solid, bottoms product relatively low in carbon, which product may be discarded, is believed readily apparent. More particularly, the need for a liquefaction process wherein a significant portion of the carbon contained in the normally solid, bottoms product can be efficiently recovered via extraction is believed to be readily apparent.

It has now been discovered that the foregoing and other disadvantages of the prior art processes can be reduced with the method of the present invention and an improved liquefaction process provided thereby. It is, therefore, an object of this invention to provide an improved liquefaction process wherein the yield of liquid product is increased without further liquefaction at elevated temperatures and pressures and without recycling the inactive and fusinite portions of the normally solid, bottom product which preferably can be discarded,directly, after an extraction operation with a reduced impact on process economics and thermal efficiency. Fusinite is the woody material which was charred before being incorporated in the peat that ultimately formed coal. The foregoing and other objects and advantages will became apparent fran the description set forth hereinafter and fran the drawings appended thereto.

In accordance with the present invention, the foregoing and other objects and advantages are accomplished by liquefying a coal or similar solid carbonaceous material in the presence of a hydrogen donor solvent at elevated temperatures and pressures and thereafter extracting at least a portion of the reactive bottoms from the normally solid bottoms product. The extraction will be accomplished with a hydrogen donor solvent derived from the solid carbonaceous material subjected to liquefaction. The raffinate from the extraction, without separation of the solvent, will be recycled to the liquefaction stage thereby increasing the overall liquid yield of the process. The normally solid bottoms product remaining after extraction will contain less carbon than the feed to the extraction step and may be discarded, directly, with less adverse impact on economics than would be the case if the original, unextracted normally solid bottoms product were discarded. As indicated more fully hereinafter, however, maximum conversion of the solid carbonaceous material and maximum thermal efficiency will be realized either by burning the remaining normally solid bottoms product or by further treating the same to produce a useful fuel.

As indicated, supra, the present invention relates to an improved process for liquefying coal and similar solid carbonaceous materials such as trash, coke and the like, wherein the yield of liquid products is increased in a more thermally efficient manner and a normally solid bottoms product containing less reactive carbon produced thereby.. The "liquefaction is accomplished at an elevated temperature and pressure and in the presence of a hydrogen donor solvent which is prepared from a portion of the liquefaction liquid product. At least a portion of the hydrogen donor solvent used during liquefaction will be used to extract the normally solid bottoms product obtained from the liquefaction and at least a portion of the carbonaceous materials extracted from the normally solid bottoms product will be present during liquefaction.

In general, the method of the present invention can be used to liquefy any solid carbonaceous material which can, effectively, be hydrogenated and liquefied. Such solid carbonaceous materials include, but are not necessarily limited to, coal, trash, biomass, coke and the like. The method of this invention is particularly useful in the liquefaction of coal and may be used to liquefy any of the coals known in the prior art including anthracite, bituminous coal, subbituminous coal, lignite, peat, brown coal and the like.

In general, the solid carbonaceous material will be ground to a finely divided state. The particular particle size or particle size range, actually employed, however, is not critical to the invention and, indeed, essentially any particle size can be employed. Notwithstanding this, generally, the solid carbonaceous material which is liquefied in accordance with this invention, will be ground to a particle size of less than 1/4 inch and preferably to a particle size of less than about 8 mesh (M.B.S.Sieve size).

. After the solid carbonaceous material has been sized, the same will be slurried with a hydrogen donor solvent. As indicated more fully hereinafter, at least a portion of the hydrogen donor solvent used in preparing the slurry will have been used to extract the normally solid bottoms product from the liquefaction step. In general, the solid carbonaceous material will be slurried with sufficient donor solvent to produce a slurry containing a solvent: solid carbonaceous material ratio within the range from about 0.8:1 to about 10:1 on a weight basis. As used herein the recitation hydrogen donor solvent shall mean a hydrogen donor solvent produced from a portion of the liquefaction liquid product and will include any non-donor species that might be contained therein.

The hydrogen donor solvent used in the process of this invention may be any portion of the liquefaction product from liquefaction containing at least about 0.8 weight percent of donatable hydrogen based on the weight of total solvent or which can be treated to contain at least about 0.8 weight percent of donatable hydrogen based on the weight of total solvent. Particularly effective solvents are distillate fractions cut from the liquefaction product and having an initial boiling point within the range from about 350°F to about 425°F and a final boiling point within the range from about 700° to about 900°F. Generally, these fractions will not contain at least about 0.8 weight percent of donatable hydrogen based on the weight of total solvent but do contain sufficient aromatic concentrations as to permit the production of a suitable hydrogen donor solvent by hydrogenating at least a portion of the aromatics to a corresponding hydroaromatic compound. In this regard, it should be noted that compounds capable of donating hydrogen during liquefaction are well-known in the prior art and many are described in U.S. Patent 3,867,275. Compounds capable of donating hydrogen during liquefaction include the indanes, the dihydroflourines, the C₁₀-C₁₂ tetra-hydro- naphathalenes, the hexahydrofluorenes, the dehydro-, tetra- hydrohexahydro-, and octohydrophenanthrenes, the C₁₂-C₁₃ acenaphthenes, the tetrahydro-, hexahydro-, and decahydro- pyrenes, the di-, tetra-, and octahydroanthracenes, and other derivatives of partially saturated aromatic compounds. As is also well-known in the prior art, hydrogenation of various coal liquefaction liquid products will produce one or more of these known hydrogen donor compounds.

During start-up of the process of this invention and while solvent produced from the solid carbonaceous materials subjected to liquefaction is not available the process may be started-up or operated with any of the known hydrogen donor compounds mentioned above. Either as a pure compound or as a mixture of such compounds either alone or in combination with components which will not donate hydrogen at liquefaction conditions. Hydrogenated creosote oil may also be used during start-up or at other times when a solvent derived from the solid carbonaceous material subject to liquefaction is not available.--Generally, the creosote oil will be hydrogenated in the same manner as is the solvent derived from the solid carbonaceous materials subjected to liquefaction, which method is described in further detail hereinafter. After the solid carbonaceous material has been slurried, the slurry will then be subjected to liquefaction at a temperature within the range from about 700 to about 950°F and at a pressure within the range from about 800 to about 3000 psig. In general, from about 20 to about 100 weight percent of the total solvent used in preparing the slurry will have first been used to extract reactive bottoms from the normally solid bottoms product produced during liquefaction. This solvent will contain from about 5 to 50 weight percent reactive bottoms. The liquefaction will, therefore, be accomplished in the presence of from about 0.05 to 0.5 parts of reactive bottoms per part of coal, based on weight. During liquefaction, the reactive bottoms will be converted to gaseous and liquid products thereby increasing the total conversion of solid carbonaceous material and the yield of normally liquid products.

During liquefaction, the solid carbonaceous material will be converted in part to a normally gaseous product, and part to a normally liquid product, and in part, to a normally solid bottoms product. In general, the normally solid bottoms product will have an initial boiling point within the range of about 900°F to about 1100°F and will contain unconverted carbonaceous material, inorganic material and high boiling but converted carbonaceous material. Generally, the high boiling, but converted carbonaceous material could be further reduced in molecular weight if the bottoms were subjected to further liquefaction or if the entire bottoms were recycled. Similarly, at least a portion of the unconverted material could be converted if the bottoms were subjected to further liquefaction or if the bottoms were recycled to a liquefaction stage. The more difficult to convert portion of the unconverted carbonaceous material (fusinite) would not, normally, be converted through further liquefaction or recycle of the bottoms. Similarly, the inorganic material (ash) would not be converted through further liquefaction of the bottoms or via recycle thereof.

It has now surprisingly been discovered that a substantial portion of the reactive material; i.e., normally solid carbonaceous material which could be converted to either a gaseous or liquid product when subjected to further liquefaction or recycled to a liquefaction stage, can be separated from the nohreactive portion of the normally solid bottoms product; viz., the ash and fusinite, by extraction of the bottoms with a donor solvent and particularly a donor solvent derived from the solid carbonaceous material being subjected to liquefaction. The extraction may be accomplished at relatively mild conditions and the extracted reactive portion of the normally solid bottoms product further converted by recycling the same to one or more of the liquefaction stages. The further conversion of the reactive portion of the normally solid bottoms product will, then, be accomplished with less energy than would be required to subject the normally solid bottoms product to further liquefaction in a separate stage and with less energy than would be required to recycle the entire normally solid bottoms product. The process of this invention is, therefore, more energy efficient than processes heretofore proposed in the prior art.

In general, the extraction will be accomplished at a temperature within the range from about 50 to about 600°F and at a pressure within the range from about 0 to about 750 psig. The extraction may be accomplished with any suitable means known in the prior art to be effective for the extraction of a soluble or extractable portion of a normally solid material with a liquid. In general, the extraction will be accomplished in a well-mixed vessel so as to ensure good contact between the normally solid bottoms product and the solvent used during extraction. The solvent containing the extracted-portion of the normally solid bottoms product can then be separated from the relatively unreactive portion of the normally solid bottoms product by any suitable means such as decanting, centrifugation, filtration or the like. Of these, decanting after a gravitational separation is most preferred since less energy is required for this particular mode of separation. Following the separation, the solvent portion may be used directly in the preparation of a slurry of the solid carbonaceous material to be subjected to liquefaction. Any solvent that might be entrained in the ash and fusinite rich raffinate stream could be removed by flash vaporization or by displacement with water. The remaining bottoms, especially when the carbon content thereof is relatively low, could be discarded. For maximum efficiency, however, it is believed most expedient to either subject the ash and fusinite rich raffinate to combustion so as to recover the fuel value thereof or to subject the same to gasification to produce a gas containing hydrogen which could then be used to effect the liquefaction and hydrogenation of the solvent fraction. When a partial oxidation process is used to effect the gasification, displacement of entrained solvent with water would offer certain advantages.

As indicated previously, the liquefaction will, generally be accomplished at a temperature within the range from about 700 to about 900°F and at a pressure within the range from about 800 to 3000 psig. Any number of liquefaction stages or zones may be used to effect the liquefaction but a single stage is generally preferred since this reduces the initial investment cost and the energy requirement for effecting the liquefaction. The total nominal holding time required is that sufficient to effect at least a partial liquefaction of the solid carbonaceous material and will, generally, range from about 10 to about 200 minutes.

As also indicated previously, the liquefaction will result in the production of a gaseous product, a normally liquid product and a normally solid bottoms product. After liquefaction, these products may be separated into respective phases using conventional techniques. For example, the gaseous products may be flashed overhead and the liquid and solids then separated using filtration, centrifugation or distillation. Of these, distillation is preferred.

After separation, the gaseous product may be upgraded to a pipeline gas or the same may be burned to provide energy for the liquefaction process. Alternatively, all or a portion of the gaseous product may be reformed to provide hydrogen for the liquefaction process.

The liquid product may be fractioned into essentially any desired product distribution and/or a portion thereof may also be used directly as a fuel or upgraded using conventional techniques. In accordance with the present invention, a portion of the liquid product will be separated and used as a solvent or diluent in the liquefaction process of this invention. This portion of the liquid product will be hydrogenated to increase the amount of donatable hydrogen therein prior to its use as a solvent or diluent. Generally, a naphtha fraction will be recovered and the naphtha fraction will be further processed to yield a high quality gasoline or similar fuel boiling in the naptha range.

Finally, in accordance with the improvement of this invention, at least a portion of the normally solid bottoms product will be withdrawn, extracted by contacting with at least a portion of the solvent separated from the liquid product and this solvent containing the extracted components from the normally solid bottoms product will be used in the preparation of a solid carbonaceous material slurry which is, ultimately, subjected to liquefaction in the process of this invention. In general, from about 1 to about 6 parts of solvent or diluent per part of normally solid bottoms product, by weight, will be contacted with the bottoms product in the extraction step. As a result of this extraction, from about 20 to about 80 weight percent of the reactive portion of the bottoms will be separated from the normally solid bottoms product during extraction. Slurry preparation will then be controlled to provide from about 0.05 to about 0.5 parts of "reactive" components per part of solid carbonaceous material fed to the liquefaction stage or zone.

In a preferred embodiment of the present invention, a coal will be liquefied in a single stage liquefaction operation in a temperature within the range from about 80 to about 880°F, and at a pressure within the range from about 1500 to about 2000 psig. In the preferred embodiment, the coal will be slurried with a solvent or diluent cut from the coal liquefaction liquid product and hydrogenated such that the solvent contains at least 45 weight percent hydrogen donor species and contains at least 1.25 weight percent donatable hydrogen. All of the solvent used in preparing the slurry will have been used to extract reactive material from the normally solid bottoms product produced during liquefaction. The slurry after preparation will contain from about 0.1 to about 0.3 parts of reactive material from the bottoms per part of coal when fed to the liquefaction stage or zone. The solvent to coal ratio in the slurry will-be within the range from about 1:1 to about 5:1. The-nominal holding time during liquefaction will be within the range from about 40 to about 140 minutes. In a preferred embodiment, the extraction will be accomplished at a temperature within the range from about 100 to about 400°F and at a pressure within the range from 0 to about 500 psig. The contacting between the solvent and the normally solid bottoms product will be accomplished in a countercurrent baffled contacting vessel at a solvent to normally solid bottoms product ratio within the range from about 4:1 to about 8:1 (v/v). In the preferred embodiment, the baffled contacting vessel will be disposed vertically with the solvent flowing upwardly-and with the normally solid bottoms product settling downwardly. The solvent will then be withdrawn at or near the top of the baffled contacting vessel and the normally solid bottoms product free of extracted reactive material will be withdrawn at or near the bottom.

It is believed that the invention will be better understood by reference to the attached Figure 1 which illustrates a particularly preferred embodiment. Referring then to Figure 1, a finely divided coal or similar solid carbonaceous material is introduced into mixing vessel 10 through line 11 and slurried with a hydrogen donor solvent or diluent introduced through line 12. In a preferred embodiment, the solvent will be all or a portion of a distillate fraction cut from the liquefaction liquid product, which fraction will be hydrogenated to produce a solvent containing at least 45 weight percent hydrogen donor species and which will be used in the extraction of reactive solid carbonaceous materials from the normally solid bottoms product. When all of the solvent is not used in the extraction step, any additional solvent required to effect the liquefaction may be recycled through line 13. During start-up, however, or when a recycle solvent is not available, any of the known useful hydrogen donor solvents or diluents may be introduced into line 13 through line 14.

In mixing vessel 10 and after normally solid bottoms product is available, the coal or similar solid carbonaceous material will also be mixed with reactive material extracted from said bottoms. In the embodiment illustrated, the reactive material will be contained in the solvent fed into mixing vessel 10 through line 12. In the preferred embodiment, the reactive material and solid carbonaceous material will be combined in a ratio within the range from about 0.1:1 to about 0.3:1 by weight. The reactive material and solid carbonaceous material will be combined with sufficient solvent including that used in the extraction step and introduced into mixing vessel 10 through line 12 to produce a slurry wherein the solvent-to-solid carbonaceous material ratio is within the range from 4:1 to about 8:1.

In the embodiment illustrated, the slurry is withdrawn from mixing vessel 10 through line 16 and passed through preheater 17. In the preheater 17 the slurry will, generally, be preheated to the desired temperature and generally to a temperature of about 50 to about 100°F below the temperature at which liquefaction is accomplished. When desired, and particularly when the solid carbonaceous material has not been previously dried, steam will be flashed overhead through line 18.

In general, the slurry of solid carbonaceous material will be combined with molecular hydrogen. In a preferred embodiment, the molecular hydrogen will be added prior to preheating through line 19. This is not, however, critical, and the hydrogen could be added downstream of preheater 17 or added directly into the liquefaction vessel. In any case, the hydrogen will be introduced after the steam is flashed overhead. In the preferred embodiment, the hydrogen will be produced either by the steam reforming of product gas from the liquefaction; by gasification of the nonreactive portion of the solid bottoms product or by gasification of solid carbonaceous material in a separate step, all in accordance with conventional technology. In general, sufficient hydrogen will be introduced to provide from about 2 to about 10 weight percent, preferably from about 3 to about 8 weight percent, molecular hydrogen based on dry, solid carbonaceous material.

The slurry is withdrawn from the preheater through line 20 and passed directly to liquefaction vessel 21. In the liquefaction vessel 21, the solid carbonaceous material is at least partially liquefied and, generally, at least partially gasified, generally, in the absence of any added catalyst. Preferably, the liquefaction vessel will be sized so as to provide a nominal holding time within the range from about 40 to about 140 minutes and in a preferred embodiment, a single vessel will be employed. Also, the temperature within the liquefaction zone-21 will, preferably, be within the range from about 800 to about 880°F and the pressure will be, preferably, controlled within the range from about 1500 to abou t 2000 psig.

In the embodiment illustrated, the combined product from liquefaction vessel 21 is withdrawn through line 22 and passed to separating means 23. In the embodiment illustrated, the separating means may be a combined atmospheric and vacuum distillation column wherein gaseous products and products boiling below the naphtha boiling range are withdrawn overhead through line 24 while a bottoms product comprising unconverted solid carbonaceous material, mineral matter and converted materials having an initial boiling point within the range from about 950°F to about 1050°F is withdrawn through line 25. The liquid product is then fractionated into desired fractions and in the embodiment illustrated, a naphtha product having an initial boiling point of about 150°F and a final boiling point within the range from about 350°F to about 425°F is withdrawn through line 26; a middle distillate fraction having an initial boiling point within the range from about 350°F to about 425°F and a final boiling point within the range from about 650°F to about 850°F is withdrawn through line 27 and a vacuum gas-oil fraction having an initial boiling point within the range from about 650°F to about 850°F and a final boiling point within the range from about 950°F to about 1050°F is withdrawn through line 28.

In general, the overhead, gaseous material will comprise gaseous and lower hydrocarbons, steam, carbon oxides, acid gases such as S0₂ and R₂S, any ammonia which may have been produced during liquefaction and any hydrogen not consumed during liquefaction. This stream may be scrubbed and further divided to yield a high Btu gas, lighter hydrocarbons and hydrogen. Generally, any hydrogen recovered from this stream will be reused in either the liquefaction or hydrogenation step. The naptha stream may be subjected to further upgrading to yield a good quality gasoline and the heavier stream/withdrawn through line 28 may be upgraded to produce a heavy fuel oil or hydrocracked and reformed to yield a gasoline boiling fraction. Generally, the solvent boiling range material or at least a portion thereof will be catalytically hydrogenated to increase the concentration of hydrogen donor species and at least a portion of the hydrogenated fraction will then be used to extract reactive material from at least a portion of the normally solid bottoms product withdrawn through line 25.

As indicated supra, the particular separation scheme employed is not critical to the present invention and, indeed, any of the separation techniques known in the prior art could be used to affect a separation of the gaseous, liquid and solid products. For example, the gaseous product could be flashed directly after liquefaction and the liquid-solid mixture then subjected to separation via distillation, filtration, extraction, centrifugation or the like. In any case, however, a bottoms product containing unreacted coal, mineral matter and high boiling hydrocarbons will be available for extraction with.a solvent separated from the liquefaction product.

In the preferred embodiment, the solvent fraction withdrawn through line 27 will be hydrogenated before the same is used either as the extraction solvent or the liquefaction solvent or diluent. Preferably, the hydrogenation Will be accomplished catalytically at conditions known to be effective for this purpose in the prior art. In the embodiment illustrated, hydrogenation is accomplished in hydrogenation vessel 29 with molecular hydrogen introduced through line 30. The hydrogen actually used may be from any source but in a preferred embodiment will be produced either through the steam reforming of at least a portion of the gaseous product from liquefaction, by gasification of at least a portion of the normally solid bottoms product or by the gasification of a portion of the solid carbonaceous material being subjected to liquefaction. In the embodiment illustrated, unreacted hydrogen and the gaseous products of hydrogenation are withdrawn through line 31. When desired, this gaseous product may be treated to recover recycle hydrogen. Also in the embodiment illustrated, the hydrogenation product is withdrawn through line 32. The hydrogenation product includes that portion of the solvent to be used in the extraction step, that portion of the solvent, if any, to be returned directly to mixing vessel 10 and any excess solvent that may have been produced. That portion of the hydrogenation product to be used as a solvent during extraction is withdrawn through line 39 and the remaining portion of the hydrogenation product is withdrawn through line 32¹. Any excess solvent may be withdrawn through line 33 as product or stored for future use during liquefaction. That portion of the solvent, if any, fed directly to mixing vessel 10 is recycled through line 13.

Normally, the hydrogenation will be accomplished at a temperature within the range from about 600°F to about 950°F and a pressure within the range from about 650 to about 2000 psig, preferably 1000 to 1500 psig. The hydrogen treat rate during the hydrogenation generally will be within the range from about 1000 to about 10,000 scf/bbl. Any of the known hydrogenation catalysts may be employed but a nickel moly catalyst is most preferred.

In accordance with the improved method of the present invention, the bottoms product withdrawn through line 25 may be divided and all or a portion thereof subjected to extraction. The portion to be subjected to extraction will be withdrawn through line 34 and fed to contacting vessel 40. In a preferred embodiment, the entire normally solid bottoms product will be passed through contacting vessel 40. Any portion of the bottoms product not subjected to extraction may be withdrawn through line 35 and processed in accordance with conventional technology. In general, from about 80 to about 100 weight percent of the bottoms product will be subjected to extraction.

In contacting vessel 40 the fraction of hydrogenated product from hydrogenation vessel 29 used as the extraction solvent is introduced at or near the bottom of contacting vessel 40 and flows upwardly through the contacting vessel and is withdrawn at or near the top thereof through line 41. The bottoms introduced through line 34 flow generally downwardly and are withdrawn from the contacting vessel at or near the bottom thereof through line 34'. In the embodiment illustrated, the solvent withdrawn through line 41 containing the extracted reactive materials is then passed through knock-out drum 42 to faciliate the separation of any unreactive materials contained-therein. The unreactive materials will be separated from knock-out drum 42 through line 43'. The unreactive materials separated in the knock-out drum may then be combined with unreactive materials separated from the contacting vessel 40 in line 43 and introduced into separator 46. In the separator, entrained solvent may be flashed overhead and the remaining portion of the normally solid bottoms product withdrawn through line 48. The recovered solvent, though, not illustrated, may be combined with solvent withdrawn from knock-out drum 42 or with solvent withdrawn from hydrogenation vessel 29 through line 32. The solvent, generally free of unreactive materials, is withdrawn from knock-out drum 42 through line 12 and fed to mixing vessel 10. The remaining portion of the normally solid bottoms product withdrawn through line 48 may be directly discarded or otherwise treated in accordance with conventional technology to recover the energy value thereof.

As indicated, supra, and in a preferred embodiment, the extraction will be accomplished at a temperature within the range from about 100 to about 400°F and at a pressure within the range from about 0 to about 500 psig. In the embodiment illustrated, the treat rate in contacting vessel 40 will be within the range from about 4 v/v/hour to 8 v/v/hour. Though not illustrated, contacting vessel 40 could be a stirred vessel and the entire solvent/normally solid bottoms product could be withdrawn and passed to a gravity separator. The major portion of the solvent could, then, be separated by withdrawing the same from the decanting vessel at a point above the solid level. Solvent entrained in the remaining solids portion could then be separated in the same manner as illustrated. When a stirred vessel is employed, space velocity is not important but sufficient contacting time should be allowed to ensure that from about 20 to about 80 weight percent of the reactive material is separated from the normally solid bottoms product. The reactive material thus separated is recovered with less energy than would be required with the use of a more conventional solvent such as toluene or the like which would, normally, be separated and reused in the extraction operation rather than as a solvent in the liquefaction step.

Having thus broadly described the present invention and a preferred embodiment thereof, it is believed that the same will become more apparent by reference to the following examples. It will be appreciated, however, that the examples are presented solely for purposes of illustration and should not be construed as limiting the invention.

### EXAMPLE 1

In this example, a run was completed in a 100 pound per day continuous unit using an Illinois seam coal (Illinois No. 6) as the solid carbonaceous material and a hydrogenated recycle liquid having an initial boiling point of about 400°F and a final boiling point of about 800°F and containing from about 40 to about 45 weight percent hydrogen donor species was used as the extraction solvent and as the solvent or diluent for liquefaction. The unit was operated in a mode similar to that illustrated in Figure 1. All of the solvent withdrawn from hydrogenation vessel 29 was used to extract bottoms from the separation vessel. As withdrawn, the bottoms contain 40 weight percent of toluene soluble material. The bottoms were extracted with the hydrogen donor solvent at 300°F and 0 psig with a nominal contacting time of 5 minutes. After extraction, the remaining portion of the normally solid bottoms product contained 10 weight percent toluene soluble material. Use of the solvent intended for slurry preparation to extract the bottoms therefore resulted in the recovery of about 75 weight percent of the reactive material from the bottoms and the gaseous and liquid product yields were increased accordingly.

### EXAMPLE'2

In this example, a run was completed in a 100 pound per day continuous unit using an Wyodak coal as the solid carbonaceous material and a hydrogenated recycle liquid having an intial boiling point of about 400°F and a final bailing point of about 800°F and containing from about 40 to about 45 weight percent hydrogen donor species was used as the extraction solvent and as the solvent or diluent for liquefaction. The unit was operated in a mode similar to that illustrated in Figure 1. All of the solvent withdrawn from hydrogenation vessel 29 was used to extract bottoms from the separation vessel. As withdrawn, the bottoms contain 50 weight percent of toluene soluble material. The bottoms were extracted with the hydrogen donor solvent at 300°F and 0 psig with a nominal contacting time of 5 minutes. After extraction, the remaining portion of the normally solid bottoms product contained 10 weight percent toluene soluble material. Use of the solvent intended for slurry preparation to extract the bottoms therefore resulted in the recovery of about 80 weight percent of the reactive material from the bottoms and the gaseous and liquid product yields were increased accordingly.

From the foregoing it will be apparent that the total conversion of the coal was increased by about 10-15 weight percent and the yield of both gaseous and liquid products was increased. This increase was, effectively, accomplished with less equipment and less energy than would have been required if an additional liquefaction stage were employed, if the entire bottoms were recycled or if a solvent had been used to extract the bottoms which would then have been separated via distillation.

## Claims

1. A process for liquefying coal or a similar solid carbonaceous material which comprises :
(a) forming a slurry of a coal or similar solid carbonaceous material in a hydrogen donor solvent;
b) subjecting the slurry from step (a) to an elevated temperature and pressure to convert the coal or similar solid carbonaceous material in part to a normally gaseous product, in part to a normally liquid product and in part to a normally solid bottoms product;
(c) separating the normally gaseous product, the normally liquid product and the normally solid bottoms product'from step (b);
(d) extracting at least a portion of the normally solid bottoms product with a donor solvent; and
(e) recycling at least a portion of the extract phase from the extraction in step (d) to the liquefaction accomplished in step (b).

2. A process according to claim 1 ₋ - in which the donor solvent is a distillate fraction separated from the liquid product obtained in step (c).

3. A process according to claim 2 in which at least a portion of the distillate fraction used as a.donor solvent is used to extract the bottoms product in step (d).

4. A process according to any one of claims 1 - 3 in which . the extract phase from the extraction of step (d) is used at least in part as the solvent used in preparing the slurry in step (a).

5. A process according to any one of claims 1 - 4 in which the extraction of step (d) is accomplished at a temperature within the range from about 50 to about 600°F and at a pressure within the range from about 0 to about 750 psig.

6. A process according to any one of claims 1 - 5 further in which the ratio of solvent to normally solid bottoms product is within the range from about 4:1 to about 8:1 v/v.

7. A liquid product whenever produced by the process of any one of claims 1 - 6.
